

June 22, 1943.

W. G. EDWARDS

2,322,288

METHOD OF TREATING CASTINGS

Filed Aug. 20, 1941



INVENTOR  
WILLIAM G. EDWARDS

BY *Ed Greenwald*  
ATTORNEY

## UNITED STATES PATENT OFFICE

2,322,288

## METHOD OF TREATING CASTINGS

William G. Edwards, Kenmore, N. Y., assignor to  
 The Linde Air Products Company, a corporation  
 of Ohio

Application August 20, 1941, Serial No. 407,544

7 Claims. (Cl. 22—216)

This invention relates to a method of thermally treating freshly poured cast bodies of metal to reduce the size of the shrinkage cavities and pipes which normally form during the solidification of the metal. More particularly, the invention concerns the treatment of steel ingots and castings risers.

Castings have been treated in the past by providing a blanket of a finely-divided carbonaceous solid fuel on the top surface of the hot casting and applying jets of air or gaseous oxygen against the blanket to burn the fuel and add heat to the top portion of the casting. In this way a pool of molten metal may be maintained in the top of the mold to feed down into the casting while solidification proceeds from the bottom toward the top, thereby inhibiting the formation of, and reducing the size and depth of, pipes and other shrinkage cavities. Finely-divided coke, coal, graphite, and charcoal have been suggested for use as the fuel.

Experience has shown that the carbonaceous fuels of the prior art, when finely divided, do not cohere under the action of flowing jets of gas but tend to blow away from the regions of gas impingement, leaving bare the top surface of the casting at those regions. Gaseous oxygen then may attack the metal directly, with the production of undesirable effects. For example, with steel castings, the oxygen may cause a "boil" in the molten metal, which may result in deep-seated porosity in the casting. Undesirable metallurgical changes in the metal likewise may be produced.

The principal object of the present invention is to provide a method of treating metal castings which will not be subject to the undesirable features of prior methods discussed above. Another object is to provide such a method characterized by the use of a carbonaceous fuel blanket which will not blow away and expose bare metal under the normal action of oxygen jets.

The above and other objects, and the novel features of the invention will become apparent from the following description, having reference to the accompanying drawing, wherein:

Fig. 1 is a vertical sectional view, taken along the line 1—1 in Fig. 2, of a large casting mold and casting with apparatus in position for performing the method of the invention; and

Fig. 2 is a plan view of the mold and apparatus of Fig. 1.

Briefly, the method of the invention comprises pouring molten metal into a mold, applying and maintaining a blanket of finely

divided lampblack on the top surface of the molten casting, impinging one or more jets of gaseous oxygen from a stationary source or sources against the blanket to cause intense combustion of the lampblack and maintain the top portion of the casting molten, and after a predetermined interval of time discontinuing the application of gaseous oxygen and permitting the metal to solidify completely in the mold.

Surprisingly, it has been found that lampblack, although light and fluffy in nature, has the property of remarkable coherence under the eroding action of a stream of gaseous oxygen. The blanket thus remains substantially intact on the top of a casting during the treatment with oxygen, except for what is actually consumed, and the residual layer of lampblack effectively insulates the metal against rapid heat loss after the oxygen flow is discontinued. Castings thus are protected against excessive upward heat loss and the consequent crusting which may result if bare steel is exposed, as well as against "boils" and excessive compositional changes which may occur during the treating period if the oxygen is permitted to come into intimate contact with bare steel. No adequate explanation for the unexpected but advantageous property of lampblack is known, although it has been suggested that the lampblack may contain a small quantity of a light binding hydrocarbon oil as a residue from its manufacture.

The remarkable coherence of a body of lampblack, coupled with its superior heat insulating property and with its relatively slow-burning even-heating nature, all combine to render the method of the invention superior to other methods known to the art.

By lampblack is meant generically the carbon collected from smoke produced by burning a hydrocarbon in insufficient air or with insufficient oxygen for complete combustion. Among the sources of lampblack are hydrocarbon oils and hydrocarbon gases, such as natural gas. The lampblack collected by the deposition on relatively cold metal surfaces of the smoke from burning hydrocarbon gases in insufficient air sometimes is known as "carbon black". The invention, of course, is not to be limited by the method of manufacture of the carbonaceous black but embraces carbonaceous black from any source which exhibits the coherent property of lampblack under an oxygen jet.

In Figs. 1 and 2 of the drawing is shown a typical arrangement of equipment for treating a

large freshly poured cast body of metal by the method of the invention. A molten steel casting 11 having a riser 12 is contained in a mold comprising a flask 13 lined with baked sand 14. A cover 15 of any suitable heat-resistant material, which covers the top of the mold and forms a substantially enclosed chamber over the top of the casting, has a plurality of ports 16 spaced from one another adjacent to the periphery of the riser 12, and a central vent and observation port 17. A rectangular header 18 resting on the top of the cover 15 is supplied with gaseous oxygen through inlets 19 and 20. A plurality of small substantially non-combustible stationary discharge tubes 21, of copper for example, take off from the header 18 and extend within the several ports 16 for discharging jets of oxygen against a blanket 22 of lampblack covering the top of the riser 12.

As soon as the molten steel has filled the mold to the desired level a layer of lampblack, which is ordinarily so finely-divided that all will pass through a screen of 325 meshes per inch, is applied to the top of the casting, the cover is placed over the mold, and the oxygen is discharged against the carbon from the stationary sources provided by the tubes 21. With this arrangement, the zone of greatest heat intensity lies close to the edges of the casting, where metal ordinarily tends to solidify first. When a large casting is treated, additional lampblack may be added to the top of the casting from time to time through the vent 17.

The number of oxygen jets required for the treatment may be varied in accordance with the size of the casting under treatment. For small risers and ingots, a single oxygen stream discharged from a single centrally arranged stationary source sometimes may be sufficient. The main requisite is that enough oxygen streams be used that the whole top surface of the casting will be kept molten and free from crusting.

Substantially pure undiluted gaseous oxygen is most efficient and produces the best results in the method of the invention, so that it is preferred despite its relatively high cost. It is evident, however, that the relatively less expensive compressed air, or oxygen-enriched air, may sometimes be used to good advantage even though it is recognized that the intensity of heating will be less.

As an example of the practical application of the method of the invention a 10,000 pound steel mill roll casting surmounted by a riser 24 inches in diameter was poured to a height 3 inches lower than previous practice and treated with 7 pounds of lampblack and 300 cu. ft. of oxygen. On sectioning the riser, 10 inches of sound steel was found above the cut-off line, being equal to or greater than the margin of safety obtained with previous practice. The saving in steel was approximately 500 pounds.

In one month 17 such steel roll castings were treated by the method of the invention with entirely successful results. The average riser diameter was 21 inches, the average oxygen consumption was 250 cu. ft., and the average amount of lampblack used was 8 pounds for each casting. The average saving in steel was 10 percent of the total weight poured, as contrasted with previous practice. 70

What is claimed is:

1. A method of treating a molten cast body of metal comprising covering the top of such cast body with a blanket of carbonaceous black, and impinging a stream of gaseous oxygen flowing from a substantially non-combustible source against said blanket, thereby burning said carbonaceous black and supplying heat to said cast body to maintain the metal fluid in the upper portion thereof.
2. A method of treating a molten cast body of metal comprising covering the top of such cast body with a blanket of lampblack, and impinging a stream of gaseous oxygen flowing from a stationary source against said lampblack, thereby burning said lampblack and supplying heat to said cast body to maintain the metal fluid in the upper portion thereof.
3. A method of treating a molten cast body of metal comprising covering the top surface of such cast body with a blanket of lampblack, and impinging a plurality of streams of gaseous oxygen against said lampblack on zones spaced from one another over the top surface of such cast body, thereby burning said lampblack and supplying heat to said cast body to maintain the metal fluid in the upper portion thereof.
4. A method of treating a molten cast body of metal comprising covering the top surface of such cast body with a blanket of lampblack, and impinging a plurality of streams of gaseous oxygen against said lampblack on zones spaced from one another and adjacent to the edges of such cast body, thereby burning said lampblack and supplying heat to said cast body to maintain the metal fluid in the upper portion thereof.
5. A method of treating a molten cast body of metal by maintaining a pool of molten metal in the upper portion thereof as solidification of the metal proceeds from the bottom toward the top, thereby feeding metal downwards and inhibiting the formation of shrinkage cavities, which method comprises: substantially enclosing the top of said casting within a chamber, applying a layer of lampblack to the top of said body, and impinging a stream of gaseous oxygen flowing from a stationary source against said lampblack, thereby burning the latter and supplying heat to said cast body.
6. A method of treating a molten cast body of metal which comprises covering the top of such molten body with a blanket of carbonaceous black having the coherence under the eroding action of a stream of gaseous oxygen, and the heat insulating and slow-burning properties, of carbon collected from smoke produced by burning a hydrocarbon with insufficient oxygen for complete combustion; and impinging gaseous oxygen flowing from at least one substantially non-combustible source against such blanket of carbonaceous black, to burn said black and thereby supply heat to the upper portion of said cast body.
7. A method of treating a molten cast body of metal as defined in claim 6, wherein substantially all of said carbonaceous black will pass through a screen of about 325 meshes per inch.

WILLIAM G. EDWARDS.